

## 1

2,977,308

## TETRAHYDRONAPHTHYLAMINO COMPOUNDS

Wilhelm Müller and Max Zimmermann, Leverkusen-Wiesdorf, and Rudolf Stroh, Leverkusen-Bayerwerk, Germany, assignors to Farbenfabriken Bayer Aktiengesellschaft, Leverkusen, Germany

No Drawing. Filed Apr. 20, 1953, Ser. No. 349,976

Claims priority, application Germany Apr. 23, 1952

2 Claims. (Cl. 252—50)

The present invention relates to compounds of the general formula



wherein X stands for a member of the group consisting of



or



R representing hydrogen or an alkyl or hydroxyalkyl radical. More particularly, the invention concerns the use of these tetrahydronaphthylamino compounds as additives to lubricants.

The tetrahydronaphthylamino compounds of the invention may be prepared by any convenient method, for instance by partially hydrogenating the corresponding naphthylamino compounds.

In general, the said tetrahydronaphthylamino compounds are oily compounds which are easily soluble in the usually employed lubricating oils. The oils provided with the new additives are very stable against oxidizing

## 2

influences; this applies particularly to oils containing tetrahydronaphthylamino compounds whose amino group is substituted by the cyclohexyl radical or by a cyclohexyl radical carrying an alkyl or hydroxyalkyl substituent. If desired, the new additives may be mixed with other additives for lubricants, for instance with additives which improve the extreme pressure properties of lubricants, particularly with phosphorus compounds described in German Patents 851,237 and 879,138. The amount of 10 the tetrahydronaphthylamino compounds to be applied as additives to lubricants can easily be determined by preliminary tests; in general, amounts of about 0.1 to 0.5% will suffice.

The following example serves to illustrate the invention, without however limiting the scope thereof.

## Example

5 parts by weight of N-cyclohexyl-tetrahydro- $\alpha$ -naphthyl-amine and 5 parts by weight of the butyl ester 20 of bis-(p-chloro-phenyl)-phosphinic acid are added to 1000 parts by weight of a refined mineral oil.

In the aging test wherein the consumption of oxygen at 150° C. in the presence of copper powder is measured by the pressure decrease by means of a mercury manometer, the oil itself and its mixture with the phosphorus compound show a pressure decrease of 100 mm. Hg within a few minutes; if however N-cyclohexyl-tetrahydro- $\alpha$ -naphthylamine is present, the consumption of oxygen is delayed to such an extent in each case that 30 this decrease in pressure occurs only after 360 minutes.

## We claim:

1. N-cyclohexyl-tetrahydro- $\alpha$ -naphthylamine.
2. A mineral oil lubricant containing N-cyclohexyl-tetrahydro- $\alpha$ -naphthylamine as an additive.

35

## References Cited in the file of this patent

## UNITED STATES PATENTS

- |           |                |                |
|-----------|----------------|----------------|
| 2,095,897 | Winans         | Oct. 12, 1937  |
| 2,109,165 | Cramer         | Feb. 22, 1938  |
| 2,131,206 | William et al. | Sept. 27, 1938 |
| 2,174,019 | Sullivan       | Sept. 26, 1939 |
| 2,633,425 | Thompson       | May 31, 1953   |

40

## FOREIGN PATENTS

- |    |         |               |               |
|----|---------|---------------|---------------|
| 45 | 276,571 | Great Britain | Sept. 1, 1927 |
|----|---------|---------------|---------------|